

## UNITED STATES PATENT OFFICE

HARRY T. BENNETT AND LE ROY G. STORY, OF TULSA, OKLAHOMA; SAID STORY AS-SIGNOR TO JOSIAH CHATFIELD, OF CLEVELAND, OHIO

## LUBRICATING OIL AND METHOD OF MAKING THE SAME

No Drawing.

Application filed October 24, 1927. Serial No. 228,487.

This invention relates to lubricating oils and methods of making the same, and more specifically to low pour point lubricating oils, which are oils that will pour at the 5 winter temperature where they are used, for example from about 10° to about 15° F. below zero.

One of the objects of the invention is to lower the pour point without impairing the 10 lubricating properties of the oil.

Another object is to obtain and maintain the low pour point. In other words, this object is to produce a lubricating oil having a stable, or fixed, low pour point which is not 15 changed by exposure to the extremes of high and low atmospheric temperatures. This object may be attained either by mixing the composition at a high temperature, or by the addition of a stabilizer when the mixture is 20 prepared at lower temperatures, as will be hereafter described.

A further object is to produce a low pour point lubricating oil without causing an objectionable change in the color of the oil.

25 A still further object is to accomplish these results by lowering the pour point without substantially changing the viscosity of the oil.

With the foregoing and other objects in 30 view, the invention comprises the novel method and product hereinafter specifically described to set forth an embodiment of the invention. However, it is to be understood that the invention comprehends changes, 35 variations and modifications which come within the scope of the claims hereunto appended.

Briefly stated, we prefer to lower the pour point by adding to a lubricating oil a quantity 40 of soap small enough to accomplish this result without materially changing the viscosity of the lubricating oil. This quantity preferably ranges between five-hundredths percent and three-tenths percent of the 45 weight of the mass, and in actual practice we have found that one-tenth percent gives highly satisfactory results. However, as will be hereafter pointed out, there is a further problem involved in maintaining or stabilizing 50 the low pour point. We have shown how this can be accomplished by the use of relatively high temperatures in the treatment of lubricating oils that will withstand such temperatures, and we have also shown how to accomplish this result by the use of 55 a stabilizer in the treatment of oils which will not withstand the relatively high temperatures.

In our early efforts to lower the pour point of a paraffin base lubricating oil, without 60 changing its viscosity, we found that the addition of very small percentages of soap, as heretofore mentioned, would produce the desired result for a more or less limited period. For example, we have prepared oils which 65 showed pour points of -10° F. but after exposure to weather temperatures ranging from 80° F. to -20° F., the pour point tended to rise and after long periods some oils even reverted to the original pour point 70 of about 15° F. to 35° F. We discovered, however, that in those cases wherein the pour point was unstable, the oils had been prepared by mixing the soap in the oil at temperatures below 300° F., whereas in every 75 case in which the soap had been mixed with the oil at temperatures in excess of 300° F. the pour point was very stable.

A temperature in excess of 300° F. for mixing the soap is suitable for some oils, such 80 as those of dark color and of rather viscous nature, but for light colored lubricating oils and certain of those of relatively low boiling points, it is desirable to maintain lower temperatures. When heating large volumes of 85 oil to elevated temperatures, a darkening of color is often experienced due to oxidation, also, expensive equipment is necessary and the operations require a relatively long time. For these reasons, it is evident that a method 90 of making stable pour points for certain oils, wherein high temperature is undesirable, would be advantageous. Thus, our process would become more flexible and broader in 95 its application, if instead of limiting it to temperatures in excess of 300° F. we could also carry out the process at lower temperatures and at the same time produce an oil having a stable or fixed low pour point. This 100

we have accomplished in a simple, inexpensive and efficient manner.

For the preparation of low pour point oils, wherein loss of color causes no serious damage or wherein the consistency is such that high temperatures are advantageous, we heat to temperatures in excess of 300° F., preferably 300 to 350° F. for the step of commingling the soap in the oil. However, in those cases wherein loss of color is a serious damage, we have discovered that the addition of an organic stabilizing agent will produce stable pour points, even when the soap is mixed with the oil at temperatures considerably below 300° F., preferably 150 to 180° F. We have found high boiling alcohols and esters such as benzyl alcohol, cyclohexanol, glycerine and benzyl acetate are particularly suitable as stabilizing agents, even in such small quantities as 0.05 to 0.2 per cent.

Our method of mixing the soap with the oil depends on the temperature we maintain. At temperatures from 300 to 350° F. we prefer to gradually add the pure soap with the oil, and to violently agitate the mass until the mixture is uniform. In this way a stable material is obtained.

At lower temperatures, for example, 150° to 180° F., in which instance a stabilizing agent is necessary, we prefer to first prepare a soap jell and to then thoroughly mix the jell with the oil. This jell may be prepared by heating a small quantity of the oil to 300 to 350° F. and incorporating therein 3 to 10 percent by weight of the soap. This latter method also produces a lubricating oil of stable pour point without heating the main body of oil to temperatures high enough to cause substantial darkening in color.

Lubricating stocks from paraffin base crudes are derived from wax distillate or namely that fraction of the crude coming from the still after the lower boiling point products such as gasoline, naphtha, kerosene and gas oil have been removed by fractional distillation. The wax distillate is essentially a mixture of paraffin wax and lubricating stock from which it is extremely difficult to remove a sufficient amount of wax to give a lubricant of pour point of 0° F. In our process it is not necessary to remove all of the wax from the oil, but only the major portion. We treat the remaining oil and wax mixture to produce a stable low pour point product.

A clearer understanding of our invention may be obtained by a more specific description of the details of one form of the invention.

A wax distillate, having a pour point of 50 to 100° F., is chilled until the major portion of the wax has separated, and the cold mixture is forced under pressure through a filter to remove the separated wax. The

filtered oil or pressed distillate, having a pour point of 20 to 35° F. is then separated by distillation into lubricating stocks of 90 to 1000 seconds Saybolt at 100° F., depending on the grade of lubricant desired. The lubricating stock is then bleached, by any of the well known methods of decolorization, such as the use of acid and clay, to the desired color, and the resulting lubricating oil heated to 150 to 180° F. One-tenth per cent of aluminum stearate in the form of a jell, is then thoroughly incorporated into the oil. After the oil and aluminum stearate are thoroughly mixed, one-tenth of one per cent of benzyl alcohol, to act as a stabilizer, is dissolved in the mixture and the mixture allowed to cool. The product has a pour point of 0 to -20° F. and is extremely stable to changing temperature conditions.

It is to be understood that we do not limit ourselves to the above example. Other soaps as well as aluminum stearate, such as aluminum palmitate, zinc stearate, zinc palmitate, etc., have given good results in amounts from five-hundredth of one percent to three-tenths of one percent. Also, the stabilizer is not limited to benzyl alcohol, as any organic stabilizer in amounts preferably ranging from five-hundredths to two-tenths of one percent may be used. As previously indicated, we wish it understood that temperatures other than those specified may be used, and that the operation of stabilizing the pour point may be performed by mixing the soap with the oil at a temperature higher than about 300° F., or by using a suitable stabilizing agent when it is necessary or desirable to employ lower temperatures.

This application is a continuation in part of the application Serial No. 98,380, filed March 29, 1926 jointly by Bennett, Story and Beckley and which related broadly to the use of minute quantities of soap for effecting the reduction in pour points of lubricating oils. This present invention provides for the treatment of crude petroleum to effect a reduction in the pour point without affecting the viscosity of the oil.

Claims for the addition of a soap to the oil while at a temperature of 300° F.-350° F. are presented in our companion and divisional application Serial No. 294,933, filed July 23, 1928.

Recognized procedure for determining pour points is provided in Technical Paper 323B, U. S. Government specification No. 2d, Department of Commerce Publication, U. S. Government Master Specification for Lubricants and Liquid Fuels and Methods for Sampling and Testing, on pages 40 and 41 of which is set forth Procedure for pour point.

We claim:

1. The method of making stable low pour point wax containing mineral lubricating oil's

- which comprises heating the oil to a temperature below 300° F., mixing therein a quantity of soap sufficient to lower the pour point without materially changing the viscosity of the oil, and stabilizing the mixture to maintain the low pour point by adding an organic stabilizing agent selected from the group consisting of benzyl alcohol, cyclo-hexanol, glycerine, and benzyl acetate.
2. The method of producing stable low pour point wax containing mineral oils, having stable pour points of 0° F. and lower, which comprises heating the oil to a temperature below 300° F., mixing therein five hundredths to three-tenths percent soap to lower the pour point without materially affecting the viscosity of the oil, and also mixing therewith an organic stabilizing agent adapted to maintain the low pour point and selected from the group consisting of benzyl alcohol, cyclo-hexanol, glycerine, and benzyl acetate.
3. The method of making stable low pour point wax containing mineral lubricating oils which comprises heating a lubricating oil composition to 150 to 180° F., mixing therein five-hundredths to three-tenths percent soap in the form of a jell and without materially affecting the viscosity of the oil, and dissolving therein five-hundredths to two-tenths per cent of an organic stabilizing agent selected from the group consisting of benzyl alcohol, cyclo-hexanol, glycerine, and benzyl acetate.
4. The method of making stable low pour point wax containing mineral lubricating oils which comprises heating a lubricating oil composition to 150 to 180° F., mixing therein about one-tenth of one percent aluminum stearate in the form of a jell and without materially affecting the viscosity of the oil, and dissolving therein five hundredths to two-tenths percent of an organic stabilizing agent selected from the group consisting of benzyl alcohol, cyclo-hexanol, glycerine, and benzyl acetate.
5. The method of making stable low pour point wax containing mineral lubricating oils which comprises heating a lubricating oil composition to 150 to 180° F., mixing therein about one-tenth percent aluminum stearate in the form of a jell, and dissolving therein about one-tenth percent benzyl alcohol.
6. The method of making a stable low pour point wax containing mineral lubricating oil which comprises removing a portion of the wax from the oil, treating the partially dewaxed product with soap to substantially lower the pour point without materially affecting the viscosity of the oil, and incorporating into the mixture an organic stabilizing agent selected from the group consisting of benzyl alcohol, cyclo-hexanol, glycerine, and benzyl acetate.
7. The method of making stable low pour point wax containing mineral lubricating oils which comprises chilling wax distillate until the major portion of the wax has crystallized, separating such portion of the wax necessary to give a dewaxed distillate of pour point 20 to 35° F., distilling said distillate to produce a lubricating stock having a viscosity of 90 to 1000 seconds Saybolt at 100° F., treating said stock to obtain the desired color, heating the resulting lubricating oil to 150 to 180° F., and mixing therein five-hundredths to three-tenths percent soap in the form of a jell and without materially affecting the viscosity of the oil, and adding to said mixture five-hundredths to two-tenths percent of an organic stabilizing agent selected from the group consisting of benzyl alcohol, cyclo-hexanol, glycerine, and benzyl acetate.
8. The method of making stable low pour point wax containing mineral lubricating oils which comprises chilling wax distillate until the major portion of the wax has crystallized, separating such portion of the wax necessary to give a dewaxed distillate of pour point 15 to 35° F., distilling said distillate to produce a lubricating stock having a viscosity of 90 to 1000 seconds Saybolt at 100° F., treating said stock to obtain the desired color, heating the resulting lubricating oil to 150 to 180° F., and mixing therein five-hundredths to three-tenths percent soap in the form of a jell, and adding to said mixture about one-tenth of one percent benzyl alcohol.
9. The method of making stable low pour point wax containing mineral lubricating oils which comprises chilling wax distillate until the major portion of the wax has crystallized, separating such portion of the wax necessary to give a dewaxed distillate of pour point 15 to 35° F., distilling said distillate to produce a lubricating stock having a viscosity of 90 to 1000 seconds Saybolt at 100° F., treating said stock to obtain the desired color, heating the resulting lubricating oil to 150 to 180° F., and mixing therein about one-tenth percent aluminum stearate in the form of a jell without materially affecting the viscosity of the oil, and adding to said mixture five-hundredths to two-tenths percent of an organic stabilizing agent selected from the group consisting of benzyl alcohol, cyclo-hexanol, glycerine, and benzyl acetate.
10. The method of making stable low pour point wax containing mineral lubricating oils which comprises chilling wax distillate until the major portion of the wax has crystallized, separating such portion of the wax necessary to give a dewaxed distillate of pour point 15 to 35° F., distilling said distillate to produce a lubricating stock having a viscosity of 90 to 1000 seconds Saybolt at 100° F., treating said stock to obtain the desired color, heating the resulting lubricating oil

to 150 to 180° F., and mixing therein about one-tenth percent aluminum stearate in the form of a jell, and adding to said mixture about one-tenth of one percent benzyl alcohol.

5 11. A stable low pour point wax-containing lubricating oil comprising a mineral lubricating oil, a minute quantity of soap whereby the low pour point is obtained, and a stabilizer whereby said pour point is maintained, the quantity of soap being small enough to produce the low pour point without materially changing the viscosity of the oil, and the stabilizer being less than two tenths percent of the mass, said stabilizer being selected from a group consisting of benzyl alcohol, cyclo-hexanol, glycerine, and benzyl acetate.

10 12. A stable low pour point lubricating oil comprising a mineral lubricating oil, a soap whereby the low pour point is obtained, and benzyl alcohol whereby said pour point is maintained, the soap being five-hundredths to three-tenths percent of the weight of the mass.

15 13. A stable low pour point wax-containing lubricating oil comprising a mineral lubricating oil, a minute quantity of soap in proportions not less than 0.05% nor more than 0.3% whereby a pour point is obtained lower than possessed by the same mineral lubricating oil without the addition of said soap, and a stabilizer whereby said low pour point is maintained, the quantity of soap being sufficiently small to produce the low pour point without materially affecting the viscosity of the oil.

20 14. A lubricating composition comprising a mineral lubricating oil having a relatively high pour point combined with aluminum stearate whereby the pour point of the oil is reduced to less than 20° F., the weight of the aluminum stearate being less than .3 percent of the weight of the mass.

25 15. A lubricating composition comprising a mineral lubricating oil having a relatively high pour point combined with aluminum stearate whereby the pour point of the oil is reduced to less than 20° F., the weight of the aluminum stearate, being about 0.1 percent of the weight of the mass.

30 16. A lubricating composition comprising a mineral lubricating oil having a relatively high pour point and a viscosity of more than 100 Saybolt at 100° F., combined with aluminum stearate whereby the pour point is reduced to about 0° F. without substantially affecting the viscosity of the oil, the weight of the aluminum stearate being about 0.1 percent of the weight of the mass.

35 60 In testimony that we claim the foregoing we hereunto affix our signatures.

HARRY T. BENNETT.  
LE ROY G. STORY.